# EUROPEAN PATENT SPECIFICATION

(11) **EP 1 392 876 B1**
(45) Date of publication and mention of the grant of the patent: **08.10.2014**
(21) Application number: 02739008.7
(22) Date of filing: 07.05.2002
(51) Int. Cl.: C22C 14/00

(54) **TITANIUM-BASE ALLOY**
TITANLEGIERUNG
ALLIAGE A BASE DE TITANE

(30) Priority: 07.05.2001 RU 2001112580
(43) Date of publication of application: 03.03.2004
(73) Proprietor: Verkhnaya Salda Metallurgical Production Association, Sverdlovsk Region, 624760 (RU); The Boeing Company, Seattle, WA 98124-2207 (US)
(72) Inventor: TETYUKHIN, Vladislav Valentinovich, Moscow, 125284 (RU); SMIRNOV, Vladimir Grigoryevich, Verkhnaya Salda, 624760 (RU); LEVIN, Igor Vasilyevich, Verkhnaya Salda, 624760 (RU)
(74) Representative: Land, Addick Adrianus Gosling
(86) International application number: PCT/RU2002/000227
(87) International publication number: WO 2002/090607

(56) References cited:
- EP-A- 0 969 109
- WO-A-01/11095
- DE-A- 19 533 743
- US-A- 4 067 734
- PATENT ABSTRACTS OF JAPAN vol. 1995, no. 05, 30 June 1995 (1995-06-30) & JP 07 054081 A (SUMITOMO METAL IND LTD), 28 February 1995 (1995-02-28)
- WELSCH,G., BOYER,R., COLLINGS,E.W.: "Materials properties handbook: titanium alloys" June 1994 (1994-06) , ASM INTERNATIONAL , MATERIALS PARK, OH44073-0002 XP002214091 page VII, paragraphs 1,2 page 165, column 1, paragraphs 2,3,5 -column 2, paragraphs 1,4 page 166 -page 168; table 1 page 263, column 1, paragraph 2 -page 264; table 1

## Description

The invention relates to the non-ferrous metallurgy, especially to the development of new titanium-base alloys offering high formability when seamless cold-worked tubes are manufactured for use in hydraulic systems of aerospace applications and sea vessels.

Due to their high strength, light weight and corrosion resistance titanium alloys are used in hydraulic systems of aerospace applications where pipe fittings are produced by welding or highly elastic pressing.

However, known titanium alloys have insufficient ductility to produce the fittings by elastic pressing.

One of known industrial titanium alloys, used in the hydraulic systems, is the alloy Ti-3Al-2.5V. This alloy features high formability during cold rolling and allows to produce fittings by elastic pressing at minimum values of yield point 515 MPa and ultimate strength 620 MPa (AMS 4943D, Seamless Annealed Pipes for Hydraulic Systems, Made of Alloy Ti-3Al-2.5V, UNSR56320).

Titanium alloy of the following composition in mass % is also known:

| | |
|---|---|
| Aluminum | 2.5 - 4.5 |
| Vanadium | 2.0 - 3.0 |
| Molybdenum | 0.5 - 2.0 |
| Zirconium | 0.5 - 2.0 |
| Iron | 0.20 max |
| Nitrogen | 0.03 max |
| Oxygen | 0.15 max |

Ref. German patent application DE 19533743 Al, Int. Cl. C22C 14/00, published 13.03.97, as prior knowledge.

This alloy is applicable for hot working, may be used for manufacture of hot-worked and seamless cold-worked pipes, possesses a favorable combination of high strength, formability and corrosion resistance but its ductility is insufficient to flare the pipe or to produce fittings by elastic pressing.

JP 07 054081 A discloses titanium alloy compositions with improved properties in regard of corrosion resistance, cold-working and welding, to be used as piping material in chemical, energy of aircraft industry. The titanium alloy comprises (in wt. %): A1 (1.5-4.5%); V (1.5-4.5%); Mo (0.1-2.5%); Zr (0.1-10%); and impurities of C, H, O, N, Fe, Y can be present in the alloy.

The object of the invention is to propose titanium alloy possessing a combination of high strength, formability and corrosion resistance, suitable for manufacture of seamless cold-worked pipes for hydraulic systems of aerospace applications and sea vessels as well as for manufacture of pipe fittings by the elastic pressing method.

In accordance with the invention this is achieved by creation of titanium-base alloy containing aluminum, vanadium, molybdenum, zirconium, iron, nitrogen and additional carbon at the following content of components, mass %:

| | |
|---|---|
| Aluminum | 2.5 - 4.0 |
| Vanadium | 2.5 - 4.0 |
| Molybdenum | 2.0 - 3.5 |
| Zirconium | 0.4 - 1.5 |
| Iron | 0.25 max |
| Nitrogen | 0.03 max |
| Oxygen | 0.15 max |
| Carbon | 0.01 - 0,1 |
| Other impurities, total | 0.3 max |
| Titanium | balance |

This titanium-base alloy may also additionally contain palladium or ruthenium in the following quantities, mass %:

| | |
|---|---|
| Palladium | 0.03 - 0.1 |
| Ruthenium | 0.03 - 0.3 |

The lower limit of the alloying element content in mass %, i.e. Al(2.5), V(2.5), Mo(2.0), Zr(0.4), of interstitial impurities Fe(0.05), N(0.005), 0(0.05) and of carbon (0.01) is the minimum at which the high strength (σ_{B} = 690 MPa, σ_{0.2} = 530 MPa) and ductility (δ = 18.4%) are ensured when the pipe diameter is expanded by the factor of 1.43 in comparison with the initial outside diameter. The high ductility during cold rolling and expansion of the pipes is achieved due to higher content of the β-phase which increases the plasticity as a result of large number of sliding planes in the crystal lattice and of the deformation of the α-phase within the β-phase under the isostatic compression.

The upper limit of the alloying element content in mass %, i.e. Al(4.0) and Zr(1.5), in combination with the maximum content of β-stabilizers V(4.0), Mo(3.5), interstitial impurities Fe(0.25), N(0.03), O(0.15), and carbon C(0.1) allows to maintain sufficient ductility (δ>17.7%) when the pipe diameter is expanded by the factor of 1.4 at high strength of the material (σ_{B} = 932 MPa, σ_{0.2} = 738 MPa).

Further increase in aluminum, zirconium and interstitial impurities content causes the increase in the α-phase quantity and strength but reduces the ductility. Increase in the β-stabilizer content reduces the alloy stability, causes grain growth during the heat treatment which also reduces the alloy ductility.

Addition of 0.01-0.1% of carbon increases the strength and ductility of the alloy and allows to use the same for manufacture of hydraulic system piping operating under severe conditions.

If the carbon content is below 0.01%, the yield point of the alloy is insufficient to ensure the performance capability of the piping in hydraulic systems. When the carbon content exceeds 0.1% the ductility of the alloy decreases at pipe expansion so that the pipe to fitting connection cannot be made by elastic pressing.

Additional alloying with palladium and ruthenium in the claimed limits increases the corrosion resistance of the alloy in the marine environment when the alloy is used in sea vessel piping.

Overalloying with the additional elements Pd and Ru in excess of the claimed limits will increase the alloy cost without any significant increase in the corrosion resistance, and underalloying below these limits cannot ensure the required corrosion resistance for long-term operation in marine environment.

Examples of the embodiment of the invention are given below.

To study the properties of the alloy, ingots with the composition shown in Table 1 have been melted in a vacuum arc furnace and pipes with the outside diameter of 1" and wall thickness of 0.051" were made from these ingots.

The mechanical and corrosion properties of the pipes are shown in Table 2.

As can be seen, the alloy with the claimed composition possesses high strength and ductility values in combination with high expansion and corrosion resistance and complies with the requirements for pipes used in hydraulic systems of aerospace applications and sea vessels.

**Table 1**

| Example | Al | V | Mo | Zr | Fe | N | C | O | Ti | Ru | Pd |
|---|---|---|---|---|---|---|---|---|---|---|---|
| 1 | 2.5 | 2.5 | 2.0 | 0.5 | 0.05 | 0.009 | 0.01 | 0.06 | base | - | - |
| 2 | 2.5 | 4.0 | 3.5 | 0.4 | 0.07 | 0.008 | 0.05 | 0.09 | base | 0.03 | - |
| 3 | 3.4 | 3.6 | 2.8 | 1.1 | 0.12 | 0.006 | 0.06 | 0.1 | base | - | - |
| 4 | 3.1 | 3.0 | 2.7 | 1.1 | 0.19 | 0.006 | 0.07 | 0.1 | base | - | 0.03 |
| 5 | 4.0 | 4.0 | 3.5 | 1.5 | 0.08 | 0.01 | 0.1 | 0.15 | base | - | - |

The outside diameter expansion was determined as the ratio of the outside diameter of the specimen after flaring to the initial outside diameter.

All specimens have sustained the test; the test was interrupted only because the support faces of the specimens lost the stability or the entire specimen lost the longitudinal stability.

## Claims

1. Titanium-base alloy containing aluminum, vanadium, molybdenum, zirconium, iron, nitrogen, wherein it additionally contains carbon, at the following content of components, mass %:
| | |
|---|---|
| Aluminum | 2.5 - 4.0 |
| Vanadium | 2.5 - 4.0 |
| Molybdenum | 2.0 - 3.5 |
| Zirconium | 0.4 - 1.5 |
| Iron | 0.25 max |
| Nitrogen | 0.03 max |
| Oxygen | 0.15 max |
| Carbon | 0.01 - 0,1 |
| Other impurities, total | 0.3 max |
wherein it additionally optionally contains palladium or ruthenium in the following quantities, mass %:
| | |
|---|---|
| Palladium | 0.03 - 0.1 |
| Ruthenium | 0.03 - 0.3 |
| Titanium | Balance |

## Patentansprüche

1. Titanlegierung, enthaltend Aluminium, Vanadium, Molybdän, Zirkonium, Eisen, Stickstoff, wobei sie zusätzlich Kohlenstoff enthält, mit dem folgenden Gehalt an Bestandteilen, Masse-%:
| | |
|---|---|
| Aluminium | 2,5 - 4,0 |
| Vanadium | 2,5 - 4,0 |
| Molybdän | 2,0 - 3,5 |
| Zirkonium | 0,4 - 1,5 |
| Eisen | 0,25 max. |
| Stickstoff | 0,03 max. |
| Sauerstoff | 0,15 max. |
| Kohlenstoff | 0,01 - 0,1 |
| sonstige Unreinheiten, insgesamt | 0,3 max., |
wobei sie zusätzlich gegebenenfalls Palladium oder Ruthenium in den folgenden Mengen enthält, Massen-%:
| | |
|---|---|
| Palladium | 0,03 - 0,1 |
| Ruthenium | 0,03 - 0,3, |
| | |
| Titan | Rest. |

## Revendications

1. Alliage à base de titane contenant de l'aluminium, du vanadium, du molybdène, du zirconium, du fer, de l'azote, et contenant en outre du carbone, avec la teneur en composants suivante, en pourcentage en masse :
| | |
|---|---|
| Aluminium | 2,5-4,0 |
| Vanadium | 2,5-4,0 |
| Molybdène | 2,0-3,5 |
| Zirconium | 0,4-1,5 |
| Fer | 0,25 max |
| Azote | 0,03 max |
| Oxygène | 0,15 max |
| Carbone | 0,01-0,1 |
| Total autres impuretés | 0,3 max |
l'alliage pouvant en outre contenir, de manière facultative, du palladium ou du ruthénium, dans les proportions suivantes, en pourcentage en masse :
| | |
|---|---|
| Palladium | 0,03-0,1 |
| Ruthénium | 0,03-0,3 |
| | |
| Titane | Reste |
